# EUROPEAN PATENT SPECIFICATION

(11) **EP 4 314 371 B1**
(45) Date of publication and mention of the grant of the patent: **29.01.2025**
(21) Application number: 22716569.3
(22) Date of filing: 29.03.2022
(51) Int. Cl.: C22C 33/04, C21C 7/00, C22C 38/02, C22C 38/04, C22C 38/12, C22C 38/24, C22C 38/26, C22C 38/46, C22C 38/48, C22C 45/02, F27B 3/02, F27B 3/08

(54) **FERROSILICON VANADIUM AND/OR NIOBIUM ALLOY, PRODUCTION OF A FERROSILICON VANADIUM AND/OR NIOBIUM ALLOY, AND THE USE THEREOF**
FERROSILICIUM-VANADIUM- UND/ODER -NIOBLEGIERUNG, HERSTELLUNG EINER FERROSILICIUM-VANADIUM- UND/ODER -NIOBLEGIERUNG UND DEREN VERWENDUNG
ALLIAGE DE FERROSILICIUM VANADIUM ET/OU NIOBIUM, PRODUCTION D'ALLIAGE DE FERROSILICIUM VANADIUM ET/OU NIOBIUM ET SON UTILISATION

(30) Priority: 30.03.2021 NO 20210413
(43) Date of publication of application: 07.02.2024
(73) Proprietor: ELKEM ASA, 0277 Oslo (NO)
(72) Inventor: KLEVAN, Ole Svein, 7507 STJØRDAL (NO); HAUNHORST, Thilo, 49076 Osnabrück (DE); OTT, Emmanuelle, 0377 OSLO (NO)
(74) Representative: Zacco Norway AS
(86) International application number: PCT/NO2022/050076
(87) International publication number: WO 2022/211640

(56) References cited:
- EP-A1- 2 717 358
- CN-A- 1 197 846
- CN-A- 101 353 751
- CN-A- 102 879 345
- CN-A- 105 886 883
- RU-C1- 2 040 575
- SU-A1- 1 399 367
- SU-A1- 1 666 568

## Description

### Technical field

The present invention relates to a ferrosilicon vanadium and/or niobium alloy, a method of production of a ferrosilicon vanadium and/or niobium alloy, and the use of such alloy. More specifically, the invention relates to a ferrosilicon vanadium and/or niobium alloy especially suitable as an additive in the manufacture of steels.

### Background art

Vanadium metal and niobium metal are known as additives to improve qualities of steels, such as finer grain size giving higher strength, increased hardenability, and higher wear resistance through precipitation of carbides and nitrides or carbonitrides. Vanadium is conventionally added to liquid steel in the form of a ferrovanadium alloy, the most common is FeV80 (80 % vanadium). Niobium is conventionally added to liquid steel in the form of a ferroniobium alloy, the most common is FeNb with 60-70 weight % niobium. In addition to iron and vanadium for ferrovanadium alloys, and iron and niobium for ferroniobium alloys, such alloys normally include small amounts of silicon, aluminium, carbon, sulfur, phosphorous, titanium, chromium, arsenic, copper and manganese, and some of these are critical impurities to steelmaking. Ferrovanadium and ferroniobium alloys have a relatively high melting temperature and therefore long dissolution times when added to a steel melt, which may lead to valuable vanadium unit or niobium unit that go into the slag instead of the steel thereby reducing the yield (also known as recovery). The conventional ways to produce ferrovanadium alloys and ferroniobium alloys are by silicon reduction and by aluminium reduction. In both methods reduction is performed in a furnace, where vanadium oxide or niobium oxide is reduced either by reaction with silicon or with aluminium. The said production methods have the disadvantages of consumption of energy to run the reaction and a relatively low vanadium yield or niobium yield as a significant amount of the vanadium oxide or niobium oxide ends up in the slag during the processing.

CN 102 879 345 B discloses a method for determining the phosphorous content of silicon ferrovanadium. A silicon ferrovanadium alloy comprising 30 - 50 wt % V, 10 - 40 wt % Si and 10 - 60 wt % Fe is disclosed.

SU 1 666 568 A1 discloses a modifier for the steel industry, containing 25.1 - 45.0 wt % V, 25.1 - 45.0 wt % Si, 20.1 - 39.0 Mn, balance iron.

CN 1 197 846 A discloses a method for smelting high-silicon and low-vanadium iron with high-vanadium iron slag and the product smelted by said method.

CN 101 353 741 A describes a vanadium-silicon alloy and its production method. The alloy contains 8 - 15 wt % V, 30- 50 wt % Si, balance iron.

EP 2 717 368 A1 relates to a negative electrode active material. Said material contains 27 to less than 100 wt % Si, more than 0 wt % to 73 wt % Sn, more than 0 to 73 wt % V and inevitable impurities.

SU 1 399 367 A1 discloses an alloy for steel containing 3 - 12 wt % RE, 20 - 35 wt % Zr, 20 - 35 wt % Si, 0.5 - 7.0 wt % Al, 0.05 - 4 wt % Mg, 0.05 - 2 wt % Ti, 0.5 - 12 wt % Cr, 0.1 - 8.0 wt % Mb, 0.3 - 5.0 wt % V, 0.05 - 5.0 Mn, balance iron.

CN 105 886 883 A discloses an inoculant for nodular cast iron, the preparation method thereof and the application of said inoculant in spheroidal graphite cast iron.

RU 2 040 575 C1 relates to a modification agent for cast iron

Therefore, there is a desire for an improved vanadium and/or niobium additive for the production of steels. It is an object of the present invention to mitigate, alleviate or eliminate one or more of the above-identified disadvantages in the prior art.

### Summary of the invention

The invention is described in the appended claims.

The present invention will become apparent from the detailed description given below. The detailed description and specific examples disclose preferred embodiments of the invention by way of illustration only. Those skilled in the art understand from guidance in the detailed description that changes and modifications may be made within the scope of the invention as defined in the appended claims.

Hence, it is to be understood that the terminology used herein is for purpose of describing particular embodiments only, and is not intended to be limiting. It should be noted that, as used in the specification and the appended claim, the articles "a", "an", "the", and "said" are intended to mean that there are one or more of the elements unless the context explicitly dictates otherwise. Furthermore, the words "comprising", "including", "containing" and similar wordings does not exclude other elements or steps.

The term "incidental impurities" should be understood to denote minor amounts of impurity elements present in the FeSi V and/ or Nb alloy or the ferrosilicon alloy, according to the normal interpretation of such term.

The term "ferrosilicon alloy" (may also be denoted "ferrosilicon", "FeSi alloy" or simply "FeSi") in the present context should be understood to be a silicon based alloy containing iron, and optionally manganese and/or chromium above impurity levels, which are conventionally produced in an submerged arc furnace (SAF) by carbothermic reduction of silica or sand with coke (or any other carbonaceous reduction agent) in the presence of iron or an iron source. Common FeSi formulations on the market are ferrosilicons with 15%, 45%, 65%, 75% and 90% (by weight) silicon. As-produced ferrosilicon alloys typically comprises about 2 wt% other elements, mainly aluminium and calcium, however, minor amounts of carbon, titanium, copper, manganese, phosphorous and sulphur are also common. The ferrosilicon alloy in the present context may also comprise manganese and/or chromium as alloying elements. Such alloys may also be denoted FeSiMn, FeSiCr and FeSiMnCr alloys. In the present context, all such possible alloys will for simplicity be referred to as ferro silicon alloys (or "ferrosilicon" "FeSi alloy" or simply "FeSi) as indicated above.

The term "ferrosilicon vanadium and/or niobium alloy" (may also be denoted "FeSi V and/or Nb alloy" or simply "FeSi V and/or Nb") in the present context should be understood to be a ferrosilicon alloy comprising vanadium or niobium or comprising both niobium and vanadium. In addition to vanadium and/or niobium, the other elements as defined in the first aspect may also be present in the alloy.

The term "up to" when used in the indication of an amount of an element in the present context should be understood to mean that the element may be present in a range from 0 wt % and up to the indicated wt % value.

### Brief descriptions of the drawings

Figure 1 is a diagram showing a comparison of dissolution time of a FeSiV10 alloy and a FeSiV20 alloy according to an embodiment of the present invention, and a standard FeV80 alloy in a steel melt.

### Detailed description

The present ferrosilicon vanadium and/or niobium (FeSi V and/or Nb) alloy is especially suitable for use as an additive in steel production for the production of vanadium and/or niobium containing steels. According to the first aspect of the present invention, it is provided a FeSi V and/or Nb alloy comprising 35 - 75 wt % Silicon (Si); 3 - 35 wt % Vanadium (V) and/or Niobium (Nb); up to 0.5 wt % Aluminium (Al); up to 25 wt % Manganese (Mn); up to 25 wt % Chromium (Cr); up to 0.15 wt % Calcium (Ca); 0.003 - 0.10 wt % Titanium (Ti); 0.003 - 0.10 wt % Carbon (C); up to 0.02 wt % Copper (Cu); up to 0.05 wt % Phosphorous (P); up to 0.02 wt % Sulfur (S); balance iron (Fe) and incidental impurities.

The present FeSi V and/or Nb alloy is especially suitable as an additive in steel manufacturing for several reasons, e.g. that the FeSi V and/or Nb alloy is low in impurities. A low aluminium content in the FeSi V and/or Nb alloy is advantageous as aluminium may cause formation of inclusions, such as for example Al₂O₃ inclusions, when added to liquid steels. These types of inclusion can be detrimental in several steels such as but not limited to spring steels and rail steels.

Further, the FeSi V and/or Nb alloy according to the present invention has a lower melting temperature and a different assimilation route in liquid steel compared with conventional FeV alloys and conventional FeNb alloys. The lower melting temperature and different assimilation route leads to significantly higher dissolution rates in liquid steel, compared to FeV and FeNb. The lower melting temperature and higher dissolution rate can lead to reduced energy consumption when added to liquid steel and may result in better distribution of vanadium and/or niobium in the melt.

Furthermore, a higher dissolution rate means that the ferrosilicon vanadium and/or niobium additive alloy can be added later in the steel manufacturing process, which may lead to less oxidizing of the vanadium and/or niobium in the steel melt. In addition, the higher dissolution rate of the alloy may prevent added lumps from resurfacing. Resurfacing enables contact between alloy and atmosphere or slag at high temperatures and can lower the yield of alloy element into steel melt. For FeSi V and/or Nb less superheat may be required for melting and dissolving into steel compared with FeV and/or FeNb which are endothermic and consume a significant amount of heat by adding into steel. Another advantage is the option to save up to two addition steps in the alloying process with the FeSi V and/or Nb alloys. This can reduce the required time in the steelmaking process and the required equipment like silos/hoppers for each alloy in the steel plant. When microalloys like FeV and/or FeNb are handled by hand due to their high cost per kilogram this effort may be saved with the usage of the lower cost per kilogram FeSi V and/or Nb alloy.

Silicon is a common additive in the manufacture of steels. Silicon is an alloying element in steel, known to increase strength, wear resistance, elasticity and scale resistance. Further, Si lowers electrical conductivity and magnetorestriction in steels. Si is also used as a treatment additive in steelmaking as a deoxidizer and slag reduction agent, commonly added as a ferrosilicon alloy. The silicon protection in FeSi V and/or Nb may be especially relevant in semi-killed steels like HSLA rebar or SBQ forging steels grades to increase the V and/or Nb yield. Further, silicon protection may allow to reduce the vacuum degassing effort for some steel grades. Lower V and/or Nb content compared to FeV and FeNb alloys together with oxidation protection by silicon may allow for less complex transportation and packing compared to prior art. Essentially, FeSi V and/or Nb may be handled in the same manner as FeSi. The amount of Si in the present FeSi V and/or Nb alloy is between 35 and 75 wt %. In an embodiment, the amount of Si is at least 40 wt %, at least 45 wt %, at least 47 wt %; or at least 51 wt %; such as at least 55 wt % or at least 58 wt %. In an embodiment, the amount of Si is up to 72 wt %; such as up to 70 wt %; or up to 68 wt %; or up to 60 wt %.

The present FeSi V and/or Nb alloy comprises between 3 and 35 wt % V and/or Nb. This means that if only V is present it may be present in the range 3 - 35 wt %. If only Nb is present it may be present in the range 3 -35 wt %. If both V and Nb are present, the total amount of V and Nb in the alloy is in the range 3 - 35 wt %. If both V and Nb are present, they may be present in any ratio of V to Nb within the given range. Vanadium and/or niobium forms stable nitrides and/or carbides and/or carbonitrides, resulting in a significant increase in the strength of steels. Steels comprising vanadium and/or niobium are such as, but not limited to, spring steels, tool steels, forging steels, rail steels, rebar steels, heavy plate steels, microalloyed automotive steels and aircraft steels. Depending on the required amounts of vanadium and/or niobium that should be added in different steel application, the content of vanadium and/or niobium in the FeSi V and/or Nb alloy may in some embodiments be in the range 5 - 30 wt %. In some embodiments, the content of vanadium and/or niobium in the FeSi V and/or Nb alloy may be at least 5 wt %, or at least 9 wt %, or at least 10 wt %; such as at least 16 wt %. In some embodiments the content of vanadium and/or niobium in the FeSi V and/or Nb alloy may be up to 25 wt%, or up to 20 wt %, or up to 15 wt %, or up to 10 wt %.

The V and/or Nb to Si range in the FeSi V and/or Nb alloy may depend on the amount of Si in the starting ferrosilicon alloy from which the FeSi V and/or Nb alloy is produced, e.g. a FeSi65 alloy might provide a higher V and/or Nb to Si range compared to when starting from e.g. a FeSi75 alloy.

In some embodiments, the FeSi V and/or Nb alloy may comprise 35-60 wt % Si and 16-35 wt % V and/or Nb, such as 16-30 wt % V and/or Nb, or such as 16-25 wt % V and/or Nb, with the other elements as defined above according to the first aspect (up to 0.5 wt % Al; up to 25 wt % Mn; up to 25 wt % Cr; up to 0.15 wt % Ca; 0.003 - 0.10 wt % Ti; 0.003 - 0.10 wt % C; up to 0.02 wt % Cu; up to 0.05 wt % P; up to 0.02 wt % S; balance Fe and incidental impurities).

In other embodiments, the FeSi V and/or Nb alloy may comprise from 51 to 75 wt % Si, such as 55 - 75 wt % Si, or 58 - 72 wt % Si, or 60 - 72 wt % Si, and from 3-35 wt % V and/or Nb, such as 5 to 30 wt % V and/or Nb, such as 5 - 25 wt % V and/or Nb, or 9 - 25 wt % V and/or Nb, or 10-20 wt % V and/or Nb, with the other elements as defined above according to the first aspect (up to 0.5 wt % Al; up to 25 wt % Mn; up to 25 wt % Cr, up to 0.15 wt % Ca; 0.003 - 0.10 wt % Ti; 0.003 - 0.10 wt % C; up to 0.02 wt % Cu; up to 0.05 wt % P; up to 0.02 wt % S; balance Fe and incidental impurities).

It should be understood that several V and/or Nb to Si ranges can be realized within the above defined alloy compositions.

The following disclosure relating to the amounts of further elements Al, Mn, Cr, Ca, Ti, C, Cu, P, S, balance Fe and incidental impurities applies to each of the above mentioned embodiments, unless otherwise stated.

The FeSi V and/or Nb alloy comprises up to 0.5 wt % Al, or, e.g., from 0.001 to 0.4 wt % Al, or from 0.01 to 0.35 wt% Al, or up to 0.2 wt % Al. In steels such as spring steels and rail steels, Al causes detrimental inclusions, such as for example Al₂O₃ inclusions. Therefore, the content of Al in the FeSi V and/or Nb alloy is preferably kept low. During the production of FeSi V and/or Nb Al in the liquid ferrosilicon will react with the oxygen of the added vanadium oxide and/or niobium oxide, resulting in a low level of Al. In alloys according to the invention, the Al content can in some embodiments be very low, for example up to only 0.04 wt %.

The FeSi V and/or Nb alloy comprises up to 25 wt % Mn. Manganese is typically an impurity in the production of ferrosilicon based alloys, and the present FeSi V and/or Nb alloy may comprise up to 0.3 wt % Mn, typically in the range 0.02 - 0.3 wt % Mn. Mn may be present as an alloying element in the starting ferrosilicon alloy when it is required as an alloying element in steel. Thus, the present FeSi V and/or Nb alloy may contain manganese in the range 0.3 - 25 wt %. Other suitable Mn ranges are 0.5-20 wt %, or 1-15 wt %, 2-12 wt % or also 3-10 wt %.

The FeSi V and/or Nb alloy comprises up to 25 wt % Cr. Chromium may be present as an impurity in the production of ferrosilicon based alloys, and the present FeSi V and/or Nb alloy may comprise up to 0.3 wt % Cr, typically in the range 0.02 - 0.3 wt % Cr. Cr may be present as an alloying element in the starting ferrosilicon alloy when it is required as an alloying element in steel. Thus, the present FeSi V and/or Nb alloy may contain chromium in the range 0.3 to 25 %. Other possible Cr ranges are 0.5-20 wt %, or 1-15 wt %, 2-12 wt % or also 3-10 wt %.

The FeSi V and/or Nb alloy comprises up to 0.15 wt % Ca, e.g., from 0.01 to 0.15 wt %. Calcium is also a common element in as-produced ferrosilicon. During the production of FeSi V and/or Nb some of the Ca in the liquid ferrosilicon will react with the oxygen of the added vanadium oxide and/or niobium oxide, resulting in a level of Ca up to about 0.15 wt %.

The FeSi V and/or Nb alloy comprises up to 0.10 wt % Ti, e.g., from 0.003 to 0.10 wt %. Titanium is normally present in low amounts in the starting ferrosilicon alloy. Titanium may also come from the vanadium oxide raw material and/or niobium oxide raw material added during the production of the FeSi V and/or Nb alloy. Titanium is harmful in some steel grades as it can form hard carbides and nitrides that lead to brittleness and reduced fatigue stress. Therefore, the content of Ti in FeSi V and/or Nb alloy is preferably as low as possible, such as below 0.025 wt %.

The FeSi V and/or Nb alloy may comprise minor amounts of C, Cu, P and S. The said elements can be normally present in small amounts in as-produced ferrosilicon or be added via the vanadium oxide raw material and/or niobium oxide raw material and/or slag modifying compound added during the production of the FeSi V and/or Nb alloy. The said elements in the indicated amounts will typically not be harmful for steel production. The FeSi V and/or Nb alloy may comprise up to 0.10 wt % C, e.g., from 0.003 to 0.10 wt % C. The FeSi V and/or Nb alloy may comprise up to 0.02 wt % Cu, e.g., 0.001 to 0.02 wt % Cu, or 0.001 to 0.01 wt %. The FeSi V and/or Nb alloy may comprise up to 0.05 wt % P, e.g., 0.001 to 0.05 wt % P. The FeSi V and/or Nb alloy may comprise up to 0.02 wt % S, e.g., 0.001 to 0.02 wt % S.

The FeSi V and/or Nb alloy, according to any of the above said embodiments, is advantageously in the form of lumps. In the present context, the term "lumps" denotes particles or pieces of the FeSi V and/or Nb alloy, e.g. of crushed FeSi V and/or Nb alloy particles. The FeSi V and/or Nb alloy lumps may be produced in different size grades. Common sizings used within steelmaking are from about 3 mm to about 80 mm. The term sizing refers to the size of the holes in a sieve that a lump fits through. It should be understood that smaller and larger sizes of the FeSi V and/or Nb lumps are possible depending on applications. Thus, the sizing may be from about 3 mm, such as from 5 mm, such as from about 10 mm, such as from about 20 mm up to about 80 mm, or up to about 50, or up to about 30 mm, or up to about 20 mm, or up to about 10 mm. Since FeSi V and/or Nb lumps are less tough than FeV and/or FeNb they may be crushed in regular FeSi crushers giving the option to produce different sizings conveniently. The FeSi V and/or Nb alloy, according to any of the above said embodiments, may also be in the form of cored wire or briquettes.

The FeSi V and/or Nb alloy, according to any of the above said embodiments, has a melting temperature range from about 1250 to about 1650 °C. The relatively low melting temperature and the assimilation route of the present FeSi V and/or Nb alloy in a steel melt has the effect that the FeSi V and/or Nb added to a steel melt dissolves relatively rapid. Tests performed by the inventors have for example shown that lumps of the FeSi V alloy according to the invention having a sizing of about 25 mm melt in about 20 seconds compared to FeV lumps dissolving only after about 60 seconds.

The method for preparing the FeSi V and/or Nb alloy according to any of the above embodiments comprises: providing a ferrosilicon alloy in liquid state in a vessel; adding a vanadium oxide containing raw material and/or a niobium oxide containing raw material to the liquid ferrosilicon alloy; mixing and reacting the liquid ferrosilicon alloy and vanadium oxide from the vanadium oxide containing raw material and/or niobium oxide from the niobium oxide containing raw material, thereby forming a melt of FeSi V and/or Nb alloy and slag; separating the slag from the said melt of FeSi V and/or Nb alloy; and solidifying or casting the liquid FeSi V and/or Nb alloy.

The reaction between the liquid ferrosilicon alloy and the vanadium oxide and/or the niobium oxide is fast allowing high productivity rate. The FeSi V and/or Nb alloy can be produced in e.g. a ladle, or a similar vessel such as a crucible or a melting pot including any kind of furnaces. As liquid FeSi in a ladle occurs in any ferrosilicon production processes there is no need of heating by supplying external energy such as using a furnace, thus allowing for economic and ecological savings over the prior art of obtaining vanadium- and/or niobium ferroalloy. The energy released from the exothermic reaction will give additional economic benefit to the FeSi production. Aluminium and calcium, which are normally present in ferrosilicon alloys (as-produced), are consumed during the reaction with vanadium oxide and/or niobium oxide, leading to a FeSi V and/or Nb alloy with very low aluminium and calcium content. Furthermore, the present method for producing the FeSi V and/or Nb alloy also leads to a high V and/or Nb-yield from the vanadium oxide and/or the niobium oxide (e.g. vanadium pentoxide and/or niobium pentoxide) added into the FeSi alloy, compared with conventional methods for producing ferrovanadium alloys, FeV and/or ferroniobium alloys, FeNb. Therefore, compared to conventional FeV and FeNb production, the present method is elegant, cost efficient, and more environmentally friendly.

The following detailed description of the method of producing FeSi V and/or Nb alloy applies to any of the above-described embodiments of the FeSi V and/or Nb alloy according to the present invention.

The liquid ferrosilicon alloy can be provided directly from a reduction furnace, typically a submerged arc furnace (SAF) wherein the ferrosilicon alloy is produced according to a conventional method. Alternatively, the liquid ferrosilicon alloy can be provided by remelting a charge of ferrosilicon, possibly refined, or a combination of as-produced ferrosilicon alloy and a solidified ferrosilicon that is brought into liquid state by any suitable heating means.

The method for preparing the FeSi V and/or Nb alloy can be performed in a ladle, or in any suitable vessel such as a crucible or a melting pot including any kind of furnaces, to hold the liquid ferrosilicon. The temperature of the ferrosilicon melt before addition of the vanadium oxide containing raw material and/or the niobium oxide containing raw material ranges ideally from about 1400 to about 1700 °C.

According to the method, the vanadium oxide containing raw material, e.g. V₂O₅, and/or niobium oxide containing raw material, e.g. Nb₂O₅, is added to the liquid ferrosilicon alloy. The vanadium oxide containing raw material and/or the niobium oxide containing raw material may be added in an amount (by weight) providing essentially the target amount of elemental vanadium and/or niobium (by weight) in the FeSi V and/or Nb alloy. The method for adding the vanadium oxide containing raw material and/or the niobium oxide containing raw material may be performed in any convenient manner that ensures contact between vanadium oxide and/or niobium oxide and liquid ferrosilicon.

The vanadium oxide containing raw material can be one or more vanadium oxide phases, such as vanadium (II) oxide, vanadium (III) oxide, vanadium (IV) oxide, vanadium (V) oxide, and/or other non-principal oxides of vanadium. The vanadium oxide is preferably vanadium (V) oxide (V₂O₅) and/or vanadium (III) oxide (V₂O₃). The vanadium oxide containing raw material may also comprise industrial waste materials or ores comprising elemental vanadium or vanadium oxide.

The niobium oxide containing raw material can be one or more niobium oxide phases, such as niobium (II) oxide, niobium (III) oxide, niobium (IV) oxide, niobium (V) oxide, and/or other non-principal oxides of niobium. The niobium oxide is preferably niobium (V) oxide (Nb₂O₅) and/or niobium (III) oxide (Nb₂O₃). The niobium oxide containing raw material may also comprise industrial waste materials or ores comprising elemental niobium or niobium oxide.

The reduction reaction of the vanadium oxide and/or the niobium oxide leads to the formation of oxide compounds, generally denoted slags. A slag modifying compound can be added to the ferrosilicon melt to modify the slag formed during the reaction. The slag modifying compound can be CaO and/or MgO, and can be added in an amount of about 0.5 - 30 wt % of the final alloy, based on the total amount of the initial ferrosilicon alloy. The necessary amount is based on the amount of vanadium oxide and/or niobium oxide to be added. The slag modifying compound can be added before or during the addition of the vanadium oxide containing raw material and/or the niobium oxide containing raw material. The slag composition is modified in a way to have a low viscosity and low melting slag to allow good slag/metal contact during the reduction reaction. Additionally, it can be modified for good metal/slag separation before casting. The slag, both produced during the reaction and added, will float on the melt, such that any formed waste and slag compounds formed during the reaction will accumulate in the layer of slag floating on the top of the melt.

The starting ferrosilicon alloy for the production of the FeSi V and/or Nb alloy should have a general composition of 45 - 90 wt % Si; up to 0.5 wt % C; up to 2 wt % Al; up to 1.5 wt % Ca; up to 0.1 wt % Ti; up to 26 wt % Mn; up to 26 wt % Cr; up to 0.02 wt % P; up to 0.005 wt % S; the balance being Fe and incidental impurities.

Examples of compositions of the starting ferrosilicon alloy are: 45 - 90 wt % Si; up to 0.5 wt % C; up to 2 wt % Al; up to 1.5 wt % Ca; up to 0.1 wt % Ti; up to 0.5 wt % Mn; up to 0.5 wt % Cr; up to 0.02 wt % P; up to 0.005 wt % S; the balance being Fe and incidental impurities;
45 - 90 wt % Si; up to 0.5 wt % C; up to 2 wt % Al; up to 1.5 wt% Ca; up to 0.1 wt % Ti; 0.5 - 26 wt % Mn; up to 0.5 wt % Cr; up to 0.02 wt % P; up to 0.005 wt % S; the balance being Fe and incidental impurities;
45 - 90 wt % Si; up to 0.5 wt % C; up to 2 wt % Al; up to 1.5 wt% Ca; up to 0.1 wt % Ti; up to 0.5 wt % Mn; 0.5 - 26 wt% Cr; up to 0.02 wt % P; up to 0.005 wt % S; the balance being Fe and incidental impurities;
45 - 90 wt % Si; up to 0.5 wt % C; up to 2 wt % Al; up to 1.5 wt% Ca; up to 0.1 wt % Ti; 0.5 - 26 wt % Mn; 0.5-26 wt% Cr; up to 0.02 wt % P; up to 0.005 wt % S; the balance being Fe and incidental impurities.

According to some embodiments of the method, the amount of Si in the starting ferrosilicon alloy is 70 - 80 wt %.

As-produced ferrosilicon alloys comprise small amounts of Al from the raw materials, typically in an amount of up to 1.5 wt %. The starting ferrosilicon alloy of the present invention may comprise up to 2 wt % Al; e.g., 0.01 - 2 wt % Al. When the vanadium oxide containing raw material and/or the niobium oxide containing raw material is added to the liquid ferrosilicon alloy, the metallic Al present in the liquid ferrosilicon reacts with the oxygen of the vanadium oxide and/or the niobium oxide reducing the vanadium and/or the niobium, resulting in pure V and/or Nb and heat while the oxidized Al will accumulate in the slag. Si in the liquid ferrosilicon alloy will also react with the oxygen of the vanadium oxide and/or the niobium oxide, resulting in reduction of vanadium oxide and/or niobium oxide to elemental V and/or Nb, while the oxidized Si will also accumulate in the slag phase. Si is less reactive than Al in the present mixture; therefore, essentially most of the Al present in the ferrosilicon alloy will react with the oxygen of the vanadium oxide and/or the niobium oxide, resulting in a very low amount of aluminium in the produced FeSi V and/or Nb alloy. Calcium is also a common element in ferrosilicon alloys, generally in an amount of up to about 1.5 wt %. Ca present in the liquid ferrosilicon alloy will also react with the oxygen of the vanadium oxide and/or the niobium oxide resulting in pure V and/or Nb and heat resulting in a low amount of Ca in the produced FeSi V and/or Nb alloy.

Additional aluminium can be added to the liquid ferrosilicon alloy, to increase the amount of Al contained in the melt available for reducing the vanadium oxide and/or the niobium oxide. This may especially be relevant when producing FeSi V and/or Nb alloy with a high amount of vanadium and/or niobium, such as from FeSi V and/or Nb with a V and/or Nb amount of 20 wt % (FeSi V and/or Nb 20), up to FeSi V and/or Nb 25 or up to FeSi V and/or Nb 30, even up to FeSi V and/or Nb 35, while keeping the amount of silicon in the FeSi V and/or Nb alloy in the upper range. If additional aluminium is added to the ferrosilicon melt, the addition can be made before, during or after, preferably during or after, the addition of the vanadium oxide containing raw material and/or the niobium oxide containing raw material. Aluminium may be added in an amount of up to about 10 wt %, or up to about 5 wt %, or up to about 1 wt %, based on the total amount of ferrosilicon and vanadium oxide and/or niobium oxide.

The liquid ferrosilicon alloy is preferably stirred during the addition of the vanadium oxide containing raw material and/or the niobium oxide containing raw material, and any added aluminium and/or slag modifying compound, and during the reduction reaction in order to ensure contact of the V and/or Nb oxides and metal. The melt is conveniently stirred by mechanical stirring and/or gas stirring means generally known in the field.

The slag can be separated before or during casting of the liquid FeSi V and/or Nb alloy. Separating the slag from the FeSi V and/or Nb melt after the reactions are completed, results in a purified FeSi V and/or Nb alloy, very low in aluminium and calcium. The FeSi V and/or Nb alloy may be casted, or solidified according to generally known methods in the field. The solidified or casted metal may be crushed and graded in size fractions adapted for different applications areas.

The FeSi V and/or Nb alloy according to the present invention may be used as an additive in the production of steels, especially as an additive for the production of vanadium containing and/or niobium containing steels. The vanadium and/or niobium containing steels may be chosen among, but not limited to, spring steels, tool steels, forging steels, rail steels, rebar steels, heavy plate steels, microalloyed automotive steels and aircraft steels.

It was surprisingly found that FeSiV and FeSiNb have a higher vanadium-yield and niobium-yield than the respective ferroalloys (FeV and FeNb). This is especially advantageous as both vanadium and niobium are scarce alloys and relatively high priced. Further, it was surprisingly found that FeSiV and FeSiNb alloys have a fast dissolution compared to the prior art alloys (FeV and FeNb). This allows the alloy elements to integrate into the steel quickly and prevents further oxidation or entrapment of V and/or Nb into the slag.

A method for production of steels, such as spring steels, tool steels, forging steels, rail steels, rebar steels, heavy plate steels, microalloyed automotive steels and aircraft steels, comprises adding a FeSi V and/or Nb alloy comprising 35 - 75 wt % Silicon (Si); 3 - 35 wt % Vanadium (V) and/or Niobium (Nb); up to 0.5 wt % Aluminium (Al); up to 25 wt % Manganese (Mn); up to 25 wt% Chromium (Cr); up to 0.15 wt % Calcium (Ca); 0.003 - 0.10 wt % Titanium (Ti); 0.003 - 0.10 wt % Carbon (C); up to 0.02 wt % Copper (Cu); up to 0.05 wt % Phosphorous (P); up to 0.02 wt % Sulfur (S); balance iron (Fe) and incidental impurities. The said method for production of steels comprises adding a FeSi V and/or Nb alloy according to any of the above-described embodiments.

### Examples

### Example 1. Production of FeSiV alloys.

Five trials for the production of FeSiV alloys according to the present invention were prepared. The following table 1 shows raw material amounts of FeSi75 and V₂O₅ for five test productions of FeSiV. Additionally, lime (CaO) amounts to modify the slag and the total Al in the system are given. The temperature (T) was set to be above the melting point of FeSiV alloy before V₂O₅ addition. The liquid ferrosilicon alloy was stirred during addition of V₂O₅, lime and any aluminium. The produced compositions are given in the right part of the table. During tapping, it is important for the purity of the produced FeSiV alloy to separate slag and metal.

**Table 1. Amounts FeSi, vanadium oxide, lime and aluminium and temperatures. Analyses of produced FeSiV alloy compositions.**

| | **Additions** | | | | | **Analyses** | | | |
|---|---|---|---|---|---|---|---|---|---|
| Test | FeSi (kg) | V₂O₅ (kg) | Lime (kg) | Al added* (kg) | T (°C) | Si (wt %) | V (wt %) | Fe (wt %) | Al (wt %) |
| 1 | 10.0 | 1.84 | 1.00 | 0.01 | 1565 | 67.1 | 9.4 | 22.8 | 0.020 |
| 2 | 7.94 | 1.46 | 0.80 | 0.11 | 1588 | 68.5 | 10.0 | 21.6 | 0.035 |
| 3 | 10.0 | 3.78 | 2.00 | 0.28 | 1585 | 58.7 | 19.2 | 21.4 | 0.024 |
| 4 | 10.0 | 1.83 | 1.00 | 0.06 | 1620 | 67.0 | 9.7 | 22.8 | 0.015 |
| 5 | 8.80 | 5.30 | 2.80 | 0.19 | 1630 | 49.7 | 29.5 | 17.8 | 0.29 |
| *AI added includes Al from FeSi and Al added separately | | | | | | | | | |

The analyses show that each of the resulting FeSiV alloys produced by the present method have a comparably low amount of aluminium. Therefore, the FeSiV alloys are very suitable as an additive in the manufacture of steels where levels of aluminium should be kept low.

Starting from FeSi alloys comprising Mn and Cr as alloying elements with Mn or Cr content of 5 wt %, 14 wt % or 25 wt %, will result in FeSi V and/or Nb alloys comprising Mn and/or Cr. This is calculated for the case of FeSiV alloys with compositions as indicated in table 2 below.

**Table 2: Amounts FeSiMn/FeSiCr, vanadium oxide, lime and resulting alloy compositions from adding V₂O₅ into FeSiMn or FeSiCr.**

| **Additions** | | | | | | | **Resulting alloy** | | | | | |
|---|---|---|---|---|---|---|---|---|---|---|---|---|
| FeSiCr/FeSiMn alloy | | | | | Lime | V₂O₅ | | | | | | |
| Si wt % | Fe wt % | Mn wt % | Cr wt % | kg | kg | kg | Kg | Si wt % | V wt % | Fe wt % | Mn wt % | Cr wt % |
| 70 | 25 | 5 | 0 | 9.7 | 1 | 1.8 | 10 | 60.9 | 10 | 24 | 4.8 | 0.0 |
| 70 | 25 | 5 | 0 | 9.4 | 2 | 3.6 | 10 | 51.9 | 20 | 23 | 4.7 | 0.0 |
| 69 | 26 | 0 | 5 | 9.7 | 1 | 1.8 | 10 | 60.9 | 10 | 24 | 0.0 | 4.8 |
| 69 | 26 | 0 | 5 | 9.4 | 2 | 3.6 | 10 | 51.9 | 20 | 23 | 0.0 | 4.7 |
| 62 | 24 | 14 | 0 | 9.7 | 1 | 1.8 | 10 | 53.2 | 10 | 23 | 13.6 | 0.0 |
| 62 | 24 | 14 | 0 | 9.4 | 2 | 3.6 | 10 | 44.4 | 20 | 23 | 13.1 | 0.0 |
| 59 | 27 | 0 | 14 | 9.7 | 1 | 1.8 | 10 | 53.2 | 10 | 23 | 0.0 | 13.6 |
| 59 | 27 | 0 | 14 | 9.4 | 2 | 3.6 | 10 | 44.4 | 20 | 23 | 0.0 | 13.1 |
| 52 | 23 | 25 | 0 | 9.7 | 1 | 1.8 | 10 | 43.5 | 10 | 22 | 24.2 | 0.0 |
| 52 | 23 | 25 | 0 | 9.4 | 2 | 3.6 | 10 | 35.0 | 20 | 22 | 23.4 | 0.0 |
| 46 | 29 | 0 | 25 | 9.7 | 1 | 1.8 | 10 | 43.5 | 10 | 22 | 0.0 | 24.2 |
| 46 | 29 | 0 | 25 | 9.4 | 2 | 3.6 | 10 | 35.0 | 20 | 22 | 0.0 | 23.4 |

Further trials for the production of FeSiV alloys according to the present invention using FeSiMn or FeSiCr as a raw material were prepared. The following table 3 shows raw material amounts of FeSiMn or FeSiCr and V₂O₅ for two test productions of FeSiV. Additionally, lime (CaO) amounts to modify the slag and the total Al in the system are given. The liquid alloy was stirred during addition of V₂O₅, lime and any aluminium. The produced compositions are given in the right part of table 3.

**Table 3: Amounts of FeSiMn/FeSiCr, lime, aluminum, V₂O₅. Analyses of produced alloy compositions.**

| **Additions** | | | | | | | | | **Analyses** | | | | |
|---|---|---|---|---|---|---|---|---|---|---|---|---|---|
| FeSiCr/FeSiMn alloy | | | | | Lime | V₂O₅ | Al | | | | | | |
| Si wt % | Fe wt % | Mn wt % | Cr wt % | kg | kg | kg | kg | T (°C) | Si wt % | V wt % | Fe wt % | Mn wt % | Cr wt % |
| 63 | 21 | 14 | | 9.7 | 1.0 | 1.8 | 0.1 | 1600 | 56 | 10 | 19 | 13 | |
| 60 | 24 | | 15 | 9.7 | 1.0 | 1.8 | 0.1 | 1650 | 53 | 10 | 23 | | 15 |

### Example 2. Production of FeSiNb alloys.

Three trials for the production of FeSiNb alloys according to the present invention were prepared. The following table 4 shows raw material amounts of FeSi75 and Nb₂O₅ for three test productions of FeSiNb. Additionally, lime (CaO) amounts to modify the slag and the total Al in the system are given. The temperature (T) was set to be above the melting point of FeSiNb alloy before Nb₂O₅ addition. The liquid ferrosilicon alloy was stirred during addition of Nb₂O₅, lime and any aluminium. The produced compositions are given in the right part of table 4. During tapping, it is important for the purity of the produced FeSiNb alloy to separate slag and metal.

**Table 4. Amounts FeSi, niobium oxide, lime and aluminium and temperatures. Analyses of produced FeSiNb alloy compositions.**

| | **Additions** | | | | | **Analyses** | | | |
|---|---|---|---|---|---|---|---|---|---|
| Test | FeSi (kg) | Nb₂O₅ (kg) | Lime (kg) | Al (kg) | T (°C) | Si (wt %) | Nb (wt %) | Fe (wt%) | Al (wt %) |
| 1 | 9 | 1.4 | 0.6 | 0.2 | 1550 | 70 | 9 | 21 | 0.25 |
| 2 | 9 | 3.1 | 1.2 | 0.5 | 1550 | 58 | 19 | 22 | 0.29 |
| 3 | 9 | 5.1 | 2.0 | 0.8 | 1650 | 47 | 32 | 21 | 0.35 |

### Example 3. Comparison of dissolution behavior of FeSiV vs. FeV80

To prove the faster dissolution behavior of FeSi V according to the present invention compared to commercial alloys as an example the dissolution behavior of a FeSiV10 (FeSiV with about 10% V) and a FeSiV20 (FeSiV with about 20% V) alloy was compared to dissolution behavior of FeV80 in a bath of low alloyed steel with a temperature of 1600 °C. The dissolution time can be measured with different techniques known from literature. Examples would be connecting a load cell to the ferroalloy and measuring the loss in weight [Argyropoulus, 1983] or taking samples of the steel melt in fixed intervals and analyzing the element content [Gourtsoyannis et al., 1984].

Fig. 1 is a diagram showing dissolution time of the FeSiV10 alloy and FeSiV20 alloy according to the present invention, compared to the standard commercial FeV80 alloy in the low-alloyed steel melt at a temperature of about 1600 °C. The diagram shows dissolution time vs. different sizing of the FeSiV10 and FeSiV20 as well as FeV80 lumps. Fig. 1 shows that the measured dissolution time for FeV80 with size 25 mm was more than 3 times longer than dissolution time of FeSiV10. The dissolution time of FeV80 alloy becomes significantly longer as the size of the lumps added to the steel melt increases, compared to the FeSiV10 and FeSiV20 alloy. A faster dissolution time shortens the steelmaking process time and thereby saves cost and increases flexibility compared to prior art solutions.

### Example 4. Yield test FeSiV10 vs. FeV80

To prove the yield behavior and the effectiveness of the alloys according to the invention to produce steel a test of FeSiV10 against FeV80 was conducted. Six steel melts of the same composition (54SiCrV6 steel) were produced in a 100 kg induction furnace at 1600 °C. The steels were deoxidized using aluminum and alloyed with the necessary alloy elements except silicon and vanadium. Three melts were alloyed using case 1: addition of FeSi75 and FeV80 and three melts were alloyed using case 2: addition of FeSiV10.

Samples of the steel melt were taken before and after the addition of the alloys and analyzed with the ICP (inductively coupled plasma) method. Additionally, solute oxygen, total oxygen, pre-alloying sample and ladle samples were analyzed to detect any possible irregularities. A comparison of the vanadium and silicon added into the melt with the vanadium and silicon analyzed in the ICP analysis was used to calculate the yields. The results are shown in table 5 below.

**Table 5: Average yields obtained from a steelmaking test with six heats of 54SiCrV6 steel.**

| | **Average Yield** | |
|---|---|---|
| Alloys | Vanadium | Silicon |
| FeSi75 + FeV80 | 90.4 % | 92.2 % |
| FeSiV10 | 93.9 % | 92.8 % |
| Improvement | + 3.5 % | + 0.6 % |

As can be seen from Table 5, it was found that the vanadium yield of FeSiV10 was on average 3.5 % higher as from FeV80. The average silicon yields are similar.

This trial proves that the present invention is not only efficiently obtaining the respective alloy element from oxides but also improves a steelmaking process by higher yield of the respective alloy.

### Example 5. Production of alloys comprising Vanadium and Niobium.

With the present invention, combined alloys of vanadium and niobium from oxides as described in table 6 can be produced. The alloys can be produced in a process of either one or two steps. The difference being that in a two-step process e.g. first FeSi V is produced from oxides with the respective ideal Al and lime addition. Then the slag is removed and the Nb is added as oxides to the liquid FeSiV with the respective ideal Al and lime additions. Subsequently the slag may be modified to help the deslagging before casting. In the same manner as described above, the alloys can be produced by starting with FeSi Nb and add V as oxides to liquid FeSiNb.

**Table 6: Amounts FeSi, vanadium oxide, niobium oxide, lime, aluminum and resulting alloy compositions.**

| **Additions** | | | | | **Resulting alloy** | | | | |
|---|---|---|---|---|---|---|---|---|---|
| FeSi (kg) | V₂O₅ (kg) | Nb₂O₅ (kg) | Lime (kg) | Al (kg) | Si (wt %) | Fe (wt %) | V (wt %) | Nb (wt %) | kg |
| 9.4 | 0.9 | 0.7 | 0.7 | 0.2 | 66 | 24 | 5 | 5 | 10 |
| 9.2 | 1.8 | 0.7 | 1.1 | 0.3 | 62 | 23 | 10 | 5 | 10 |
| 9.1 | 0.9 | 1.4 | 0.9 | 0.3 | 62 | 23 | 5 | 10 | 10 |
| 8.9 | 1.8 | 1.4 | 1.4 | 0.4 | 58 | 22 | 10 | 10 | 10 |
| 8.7 | 2.7 | 1.4 | 1.8 | 0.4 | 53 | 22 | 15 | 10 | 10 |
| 8.5 | 1.8 | 2.1 | 1.6 | 0.5 | 54 | 21 | 10 | 15 | 10 |
| 9.0 | 2.7 | 0.7 | 1.6 | 0.3 | 57 | 23 | 15 | 5 | 10 |
| 8.7 | 0.9 | 2.1 | 1.1 | 0.4 | 58 | 22 | 5 | 15 | 10 |
| 8.3 | 2.7 | 2.1 | 2.0 | 0.6 | 49 | 21 | 15 | 15 | 10 |
| 8.5 | 3.6 | 1.4 | 2.2 | 0.5 | 49 | 21 | 20 | 10 | 10 |
| 8.1 | 1.8 | 2.9 | 1.8 | 0.6 | 50 | 20 | 10 | 20 | 10 |
| 7.7 | 3.6 | 2.9 | 2.7 | 0.8 | 41 | 19 | 20 | 20 | 10 |

### Example 6. Production of FeSiVNb alloys.

A trial for the production of a FeSiVNb alloy according to the present invention was prepared. The following table 7 shows raw material amounts of FeSi75, V₂O₅, and Nb₂O₅ for a test production of FeSiVNb. Additionally, lime (CaO) amounts to modify the slag and the total Al in the system are given. The temperature (T) was set to be above the melting point of FeSiVNb alloy before any oxide addition. The liquid ferrosilicon alloy was stirred during addition of V₂O₅, Nb₂O₅, lime and any aluminium. The produced composition is given in the right part of table 7. During tapping, it is important for the purity of the produced FeSiVNb alloy to separate slag and metal.

**Table 7. Amounts FeSi, vanadium oxide, niobium oxide, lime and aluminium and temperature. Analyses of produced FeSiVNb alloy composition.**

| **Additions** | | | | | | **Analyses** | | | | |
|---|---|---|---|---|---|---|---|---|---|---|
| FeSi (kg) | V₂O₅ (kg) | N₂O₅ (kg) | Lime (kg) | Al (kg) | T (°C) | Si (wt%) | V (wt%) | Nb (wt%) | Fe (wt%) | Al (wt%) |
| 9.0 | 1.93 | 1.51 | 1.68 | 0.44 | 1700 | 57 | 8.8 | 10.6 | 23 | 0.1 |

The person skilled in the art realizes that the present invention is not limited to the preferred embodiments described above. The person skilled in the art further realizes that modifications and variations are possible within the scope of the appended claims. Additionally, variations to the disclosed embodiments can be understood and effected by the skilled person in practicing the claimed invention, from a study of the disclosure, and the appended claims.

## Claims

1. A ferrosilicon vanadium and/or niobium, FeSi V and/or Nb, alloy, comprising
35 - 75 wt % Si;
3 - 35 wt % V and/or Nb;
up to 0.5 wt % Al;
up to 25 wt % Mn;
up to 25 wt % Cr;
up to 0.15 wt % Ca;
0.003 - 0.10 wt % Ti;
0.003 - 0.10 wt % C;
up to 0.02 wt % Cu;
up to 0.05 wt % P;
up to 0.02 wt % S;
balance Fe and incidental impurities.

2. The FeSi V and/or Nb alloy according to claim 1, comprising 35 - 60 wt % Si; 16 - 35 wt % V and/or Nb; up to 0.5 wt % Al; up to 25 wt % Mn; up to 25 wt% Cr; up to 0.15 wt % Ca; 0.003 - 0.10 wt % Ti; 0.003 - 0.10 wt % C; up to 0.02 wt % Cu; up to 0.05 wt % P; up to 0.02 wt% S; balance Fe and incidental impurities.

3. The FeSi V and/or Nb alloy according to claim 1, comprising 51 - 75 wt % Si; 3 - 35 wt % V and/or Nb; up to 0.5 wt % Al; up to 25 wt % Mn; up to 25 wt% Cr; up to 0.15 wt % Ca; 0.003 - 0.10 wt % Ti; 0.003 - 0.10 wt % C; up to 0.02 wt % Cu; up to 0.05 wt % P; up to 0.02 wt % S; balance Fe and incidental impurities.

4. The FeSi V and/or Nb alloy according to any one of claims 1 or 3, comprising 5 - 25 wt % V and/or Nb.

5. The FeSi V and/or Nb alloy according to any one of claims 1, 3 or 4, comprising 60 - 72 wt % Si.

6. The FeSi V and/or Nb alloy according to any one of claims 1-5, comprising up to 0.025 wt % Ti.

7. The FeSi V and/or Nb alloy according to any one of claims 1-6, comprising up to 0.3 wt % Mn.

8. The FeSi V and/or Nb alloy according to any one of claims 1-6, comprising 0.3 - 25 wt % Mn.

9. The FeSi V and/or Nb alloy according to any one of claims 1-8, comprising up to 0.3 wt % Cr.

10. The FeSi V and/or Nb alloy according to any one of claims 1-8, comprising 0.3 - 25 wt % Cr.

11. The FeSi V and/or Nb alloy according to any one of claims 1-10, wherein the FeSi V and/or Nb alloy has a melting temperature range from 1250 to 1650 °C.

12. The FeSi V and/or Nb alloy according to any one of claims 1-11, wherein the FeSi V and/or Nb alloy is in the form of particles or lumps having a sizing of 3 mm to 80 mm or in the form of cored wire or in the form of briquettes.

13. The FeSi V and/or Nb alloy according to any one of claims 1-12, wherein the FeSi V and/or Nb alloy is an additive for use in production of steels.

14. A method for production of a ferrosilicon vanadium and/or niobium (FeSi V and/or Nb) alloy according to any one of claims 1-13, the method comprises:
- providing a ferrosilicon alloy in liquid state in a vessel;
- adding vanadium oxide containing raw material and/or niobium oxide containing raw material to the liquid ferrosilicon alloy, where the vanadium oxide containing raw material and/or the niobium oxide containing raw material is added in an amount (by weight) providing essentially the target amount of elemental vanadium and/or niobium (by weight) in the FeSi V and/or Nb alloy;
- mixing and reacting the liquid ferrosilicon alloy and vanadium oxide from the vanadium oxide containing raw material and/or niobium oxide from the niobium oxide containing raw material, thereby forming a melt of FeSi V and/or Nb alloy and slag;
- separating the slag from the said melt; and
- solidifying or casting the liquid FeSi V and/or Nb alloy.

15. The method according to claim 14, where the liquid ferrosilicon alloy is provided directly from a reduction furnace, wherein ferrosilicon is as-produced from raw materials according to conventional methods.

16. The method according to claim 14, where the liquid ferrosilicon alloy is provided by remelting a charge of ferrosilicon alloy.

17. The method according to any one of claims 14-16, where the vanadium oxide containing raw material is one or more vanadium oxide phases selected from vanadium(II) oxide, vanadium(III) oxide, vanadium(IV) oxide, vanadium(V) oxide, and/or other non-principal oxides of vanadium and/or the niobium oxide containing raw material is one or more niobium oxide phases selected from niobium(II) oxide, niobium(III) oxide, niobium(IV) oxide, niobium(V) oxide, and/or other non-principal oxides of niobium.

18. The method according to claim 17, where the vanadium oxide phase is vanadium(V) oxide, V₂O₅ and/or vanadium(III) oxide, V₂O₃ and/or the niobium oxide phase is niobium(V) oxide, Nb₂O₅ and/or niobium(III) oxide, Nb₂O₃.

19. The method according to claim 17 or 18, wherein the vanadium oxide containing raw material further comprises industrial waste material or ore comprising elemental vanadium or vanadium oxide, and/or the niobium oxide containing raw material further comprises industrial waste material or ore comprising elemental niobium or niobium oxide.

20. The method according to any one of claims 14-19, further comprising adding a slag modifying compound to the liquid ferrosilicon alloy in an amount of 0.5 - 30 wt %, based on the total amount of ferrosilicon alloy.

21. The method according to claim 20, where the slag modifying compound is at least one of CaO and MgO.

22. The method according to any one of claims 14-21, where the liquid starting ferrosilicon alloy has a general composition;
45 - 90 wt % Si;
up to 0.5 wt % C;
up to 2 wt % Al;
up to 1.5 wt% Ca;
up to 0.1 wt % Ti;
up to 26 wt % Mn;
up to 26 wt % Cr;
up to 0.02 wt % P;
up to 0.005 wt % S;
the balance being Fe and incidental impurities.

23. The method according to any one of claims 14-22, further comprising adding aluminium to the ferrosilicon melt, prior to, simultaneously, or after the addition of the vanadium oxide containing raw material and/or the niobium oxide containing raw material, in an amount of up to 10 wt %, based on the total amount of ferrosilicon and vanadium oxide and/or niobium oxide.

24. The method according to any one of claims 14-23, comprising mixing the liquid ferrosilicon alloy and the vanadium oxide containing raw material and/or the niobium oxide containing raw material, and any added aluminium and/or slag modifying compound, by mechanical stirring or gas stirring.

25. The method according to any one of claims 14-24, where the slag is separated before or during casting of the liquid FeSi V and/or Nb alloy.

26. The method according to any one of claims 14-25, further comprising crushing, and optionally grading in size fractions, the solidified or casted FeSi V and/or Nb alloy.

27. Use of a FeSi V and/or Nb alloy, according to any one of claims 1-13, as an additive in the manufacture of vanadium and/or niobium containing steels.

28. Use according to claim 27, where the vanadium and/or niobium containing steels are chosen among spring steels, tool steels, forging steels, rail steels, rebar steels, heavy plate steels, microalloyed automotive steels and aircraft steels.

## Patentansprüche

1. Ferrosilicium-Vanadium- und/oder -Nioblegierung, FeSiV- und/oder -Nb-Legierung, umfassend
35-75 Gew.-% Si;
3-35 Gew.-% V und/oder Nb;
bis zu 0,5 Gew.-% Al;
bis zu 25 Gew.-% Mn;
bis zu 25 Gew.-% Cr;
bis zu 0,15 Gew.-% Ca;
0,003-0,10 Gew.-% Ti;
0,003-0,10 Gew.-% C;
bis zu 0,02 Gew.-% Cu;
bis zu 0,05 Gew.-% P;
bis zu 0,02 Gew.-% S;
Rest Fe und zufällige Verunreinigungen.

2. FeSiV- und/oder -Nb-Legierung nach Anspruch 1, umfassend 35-60 Gew.-% Si; 16-35 Gew.-% V und/oder Nb; bis zu 0,5 Gew.-% Al; bis zu 25 Gew.-% Mn; bis zu 25 Gew.-% Cr; bis zu 0,15 Gew.-% Ca; 0,003-0,10 Gew.-% Ti; 0,003-0,10 Gew.-% C; bis zu 0,02 Gew.-% Cu; bis zu 0,05 Gew.-% P; bis zu 0,02 Gew.-% S; Rest Fe und zufällige Verunreinigungen.

3. FeSiV- und/oder -Nb-Legierung nach Anspruch 1, umfassend 51-75 Gew.-% Si; 3-35 Gew.-% V und/oder Nb; bis zu 0,5 Gew.-% Al; bis zu 25 Gew.-% Mn; bis zu 25 Gew.-% Cr; bis zu 0,15 Gew.-% Ca; 0,003-0,10 Gew.-% Ti; 0,003-0,10 Gew.-% C; bis zu 0,02 Gew.-% Cu; bis zu 0,05 Gew.-% P; bis zu 0,02 Gew.-% S; Rest Fe und zufällige Verunreinigungen.

4. FeSiV- und/oder -Nb-Legierung nach einem der Ansprüche 1 oder 3, umfassend 5-25 Gew.-% V und/oder Nb.

5. FeSiV- und/oder -Nb-Legierung nach einem der Ansprüche 1, 3 oder 4, umfassend 60-72 Gew.-% Si.

6. FeSiV- und/oder -Nb-Legierung nach einem der Ansprüche 1-5, umfassend bis zu 0,025 Gew.-% Ti.

7. FeSiV- und/oder -Nb-Legierung nach einem der Ansprüche 1-6, umfassend bis zu 0,3 Gew.-% Mn.

8. FeSiV- und/oder -Nb-Legierung nach einem der Ansprüche 1-6, umfassend 0,3-25 Gew.-% Mn.

9. FeSiV- und/oder -Nb-Legierung nach einem der Ansprüche 1-8, umfassend bis zu 0,3 Gew.-% Cr.

10. FeSiV- und/oder -Nb-Legierung nach einem der Ansprüche 1-8, umfassend 0,3-25 Gew.-% Cr.

11. FeSiV- und/oder -Nb-Legierung nach einem der Ansprüche 1-10, wobei die FeSiV- und/oder -Nb-Legierung einen Schmelztemperaturbereich von 1250 bis 1650 °C aufweist.

12. FeSiV- und/oder -Nb-Legierung nach einem der Ansprüche 1-11, wobei die FeSiV- und/oder -Nb-Legierung in Form von Partikeln oder Klumpen, die eine Größe von 3 mm bis 80 mm aufweisen, oder in Form von Fülldraht oder in Form von Briketts vorliegt.

13. FeSiV- und/oder -Nb-Legierung nach einem der Ansprüche 1-12, wobei die FeSiV- und/oder -Nb-Legierung ein Zusatzstoff zur Verwendung bei der Herstellung von Stahl ist.

14. Verfahren zur Herstellung einer Ferrosilicium-Vanadium- und/oder -Nioblegierung (FeSiV und/oder -Nb-Legierung) nach einem der Ansprüche 1-13, wobei das Verfahren Folgendes umfasst:
- Bereitstellen einer Ferrosiliciumlegierung in einem flüssigen Zustand in einem Gefäß;
- Hinzufügen eines vanadiumoxidhaltigen Rohmaterials und/oder eines nioboxidhaltigen Rohmaterials zu der flüssigen Ferrosiliciumlegierung, wobei das vanadiumoxidhaltige Rohmaterial und/oder das nioboxidhaltige Rohmaterial in einer Menge (nach Gewicht) hinzugefügt werden, die im Wesentlichen die Zielmenge an elementarem Vanadium und/oder Niob (nach Gewicht) in der FeSiV- und/oder -Nb-Legierung bereitstellt;
- Mischen und Umsetzen der flüssigen Ferrosiliciumlegierung und des Vanadiumoxids aus dem vanadiumoxidhaltigen Rohmaterial und/oder des Nioboxids aus dem nioboxidhaltigen Rohmaterial, wodurch eine Schmelze aus FeSiV- und/oder -Nb-Legierung und Schlacke gebildet wird;
- Trennen der Schlacke von der Schmelze; und
- Verfestigen oder Gießen der flüssigen FeSiV- und/oder -Nb-Legierung.

15. Verfahren nach Anspruch 14, wobei die flüssige Ferrosiliciumlegierung direkt aus einem Reduktionsofen bereitgestellt wird, wobei Ferrosilicium nach herkömmlichen Verfahren aus Rohmaterialien hergestellt ist.

16. Verfahren nach Anspruch 14, wobei die flüssige Ferrosiliciumlegierung durch erneutes Schmelzen einer Charge Ferrosiliciumlegierung bereitgestellt wird.

17. Verfahren nach einem der Ansprüche 14-16, wobei es sich bei dem vanadiumoxidhaltigen Rohmaterial um eine oder mehrere Vanadiumoxidphasen handelt, die ausgewählt sind aus Vanadium(II)-oxid, Vanadium(III)-oxid, Vanadium(IV)-oxid, Vanadium(V)-oxid und/oder anderen Nebenoxiden von Vanadium, und/oder es sich bei dem nioboxidhaltigen Rohmaterial um eine oder mehrere Nioboxidphasen handelt, die ausgewählt sind aus Niob(II)-oxid, Niob(III)-oxid, Niob(IV)-oxid, Niob(V)-oxid und/oder anderen Nebenoxiden von Niob.

18. Verfahren nach Anspruch 17, wobei es sich bei der Vanadiumoxidphase um Vanadium(V)-oxid, V₂O₅, und/oder Vanadium(III)-oxid, V₂O₃, handelt und/oder es sich bei der Nioboxidphase um Niob(V)-oxid, Nb₂O₅ und/oder Niob(III)-oxid, Nb₂O₃, handelt.

19. Verfahren nach Anspruch 17 oder 18, wobei das vanadiumoxidhaltige Rohmaterial ferner Industrieabfallmaterial oder Erz umfasst, das elementares Vanadium oder Vanadiumoxid umfasst, und/oder das nioboxidhaltige Rohmaterial ferner Industrieabfallmaterial oder Erz umfasst, das elementares Niob oder Nioboxid umfasst.

20. Verfahren nach einem der Ansprüche 14-19, ferner umfassend Hinzufügen einer schlackemodifizierenden Verbindung zu der flüssigen Ferrosiliciumlegierung in einer Menge von 0,5-30 Gew.-%, basierend auf der Gesamtmenge an Ferrosiliciumlegierung.

21. Verfahren nach Anspruch 20, wobei die schlackemodifizierende Verbindung mindestens eines von CaO und MgO ist.

22. Verfahren nach einem der Ansprüche 14-21, wobei die flüssige Ausgangsferrosiliciumlegierung eine allgemeine Zusammensetzung aufweist;
45-90 Gew.-% Si;
bis zu 0,5 Gew.-% C;
bis zu 2 Gew.-% Al;
bis zu 1,5 Gew.-% Ca;
bis zu 0,1 Gew.-% Ti;
bis zu 26 Gew.-% Mn;
bis zu 26 Gew.-% Cr;
bis zu 0,02 Gew.-% P;
bis zu 0,005 Gew.-% S;
der Rest sind Fe und zufällige Verunreinigungen.

23. Verfahren nach einem der Ansprüche 14-22, ferner umfassend Hinzufügen von Aluminium zu der Ferrosiliciumschmelze vor dem, gleichzeitig zum oder nach dem Hinzufügen des vanadiumoxidhaltigen Rohmaterials und/oder des nioboxidhaltigen Rohmaterials in einer Menge von bis zu 10 Gew.-%, basierend auf der Gesamtmenge an Ferrosilicium und Vanadiumoxid und/oder Nioboxid.

24. Verfahren nach einem der Ansprüche 14-23, umfassend Mischen der flüssigen Ferrosiliciumlegierung und des vanadiumoxidhaltigen Rohmaterials und/oder des nioboxidhaltigen Rohmaterials und einer beliebigen hinzugefügten Aluminium- und/oder schlackemodifizierenden Verbindung durch mechanisches Rühren oder Gasrühren.

25. Verfahren nach einem der Ansprüche 14-24, wobei die Schlacke vor oder während des Gießens der flüssigen FeSiV- und/oder -Nb-Legierung getrennt wird.

26. Verfahren nach einem der Ansprüche 14-25,ferner umfassend Zerkleinern und optional Sortieren in Größenfraktionen der verfestigten oder gegossenen FeSiV- und/oder -Nb-Legierung.

27. Verwendung einer FeSiV- und/oder -Nb-Legierung nach einem der Ansprüche 1-13 als Zusatzstoff bei der Herstellung von vanadium- und/oder niobhaltigen Stählen.

28. Verwendung nach Anspruch 27, wobei die vanadium- und/oder niobhaltigen Stähle ausgewählt sind aus Federstählen, Werkzeugstählen, Schmiedestählen, Schienenstählen, Betonstahlstählen, Grobblechstählen, mikrolegierten Automobilstählen und Flugzeugstählen.

## Revendications

1. Alliage de ferrosilicium vanadium et/ou niobium, FeSi V et/ou Nb, comprenant
35 à 75 % en poids de Si ;
3 à 35 % en poids de V et/ou de Nb ;
jusqu'à 0,5 % en poids d'Al ;
jusqu'à 25 % en poids de Mn ;
jusqu'à 25 % en poids de Cr ;
jusqu'à 0,15 % en poids de Ca ;
0,003 à 0,10 % en poids de Ti ;
0,003 à 0,10 % en poids de C ;
jusqu'à 0,02 % en poids de Cu ;
jusqu'à 0,05 % en poids de P ;
jusqu'à 0,02 % en poids de S ;
le reste étant du Fe et des impuretés accidentelles.

2. Alliage FeSi V et/ou Nb selon la revendication 1, comprenant 35 à 60 % en poids de Si ; 16 à 35 % en poids de V et/ou de Nb ; jusqu'à 0,5 % en poids d'Al ; jusqu'à 25 % en poids de Mn ; jusqu'à 25 % en poids de Cr ; jusqu'à 0,15 % en poids de Ca ; 0,003 à 0,10 % en poids de Ti ; 0,003 à 0,10 % en poids de C ; jusqu'à 0,02 % en poids de Cu ; jusqu'à 0,05 % en poids de P ; jusqu'à 0,02 % en poids de S ; le reste étant du Fe et des impuretés accidentelles.

3. Alliage FeSi V et/ou Nb selon la revendication 1, comprenant 51 à 75 % en poids de Si ; 3 à 35 % en poids de V et/ou de Nb ; jusqu'à 0,5 % en poids d'Al ; jusqu'à 25 % en poids de Mn ; jusqu'à 25 % en poids de Cr ; jusqu'à 0,15 % en poids de Ca ; 0,003 à 0,10 % en poids de Ti ; 0,003 à 0,10 % en poids de C ; jusqu'à 0,02 % en poids de Cu ; jusqu'à 0,05 % en poids de P ; jusqu'à 0,02 % en poids de S ; le reste étant du Fe et des impuretés accidentelles.

4. Alliage FeSi V et/ou Nb selon l'une quelconque des revendications 1 ou 3, comprenant 5 à 25 % en poids de V et/ou de Nb.

5. Alliage FeSi V et/ou Nb selon l'une quelconque des revendications 1, 3 ou 4, comprenant 60 à 72 % en poids de Si.

6. Alliage FeSi V et/ou Nb selon l'une quelconque des revendications 1 à 5, comprenant jusqu'à 0,025 % en poids de Ti.

7. Alliage FeSi V et/ou Nb selon l'une quelconque des revendications 1 à 6, comprenant jusqu'à 0,3 % en poids de Mn.

8. Alliage FeSi V et/ou Nb selon l'une quelconque des revendications 1 à 6, comprenant 0,3 à 25 % en poids de Mn.

9. Alliage FeSi V et/ou Nb selon l'une quelconque des revendications 1 à 8, comprenant jusqu'à 0,3 % en poids de Cr.

10. Alliage FeSi V et/ou Nb selon l'une quelconque des revendications 1 à 8, comprenant 0,3 à 25 % en poids de Cr.

11. Alliage FeSi V et/ou Nb selon l'une quelconque des revendications 1 à 10, dans lequel l'alliage FeSi V et/ou Nb a une plage de température de fusion de 1250 à 1650°C.

12. Alliage FeSi V et/ou Nb selon l'une quelconque des revendications 1 à 11, dans lequel l'alliage FeSi V et/ou Nb se présente sous la forme de particules ou de morceaux ayant une taille de 3 mm à 80 mm ou sous la forme de fil fourré ou sous la forme de briquettes.

13. Alliage FeSi V et/ou Nb selon l'une quelconque des revendications 1 à 12, dans lequel l'alliage FeSi V et/ou Nb est un additif destiné à être utilisé dans la production d'aciers.

14. Procédé de production d'un alliage de ferrosilicium vanadium et/ou niobium (FeSi V et/ou Nb) selon l'une quelconque des revendications 1 à 13, le procédé comprenant :
- la fourniture d'un alliage de ferrosilicium à l'état liquide dans un récipient ;
- l'ajout d'une matière première contenant de l'oxyde de vanadium et/ou de l'oxyde de niobium à l'alliage de ferrosilicium liquide, la matière première contenant de l'oxyde de vanadium et/ou la matière première contenant de l'oxyde de niobium étant ajoutée en une quantité (en poids) fournissant essentiellement la quantité cible de vanadium et/ou de niobium élémentaire (en poids) dans l'alliage FeSi V et/ou Nb ;
- le mélange et la réaction de l'alliage de ferrosilicium liquide et l'oxyde de vanadium provenant de la matière première contenant de l'oxyde de vanadium et/ou l'oxyde de niobium provenant de la matière première contenant de l'oxyde de niobium, formant ainsi une masse fondue d'alliage FeSi V et/ou Nb et de scories ;
- la séparation des scories de ladite masse fondue ; et
- la solidification ou la coulée de l'alliage de liquide FeSi V et/ou Nb.

15. Procédé selon la revendication 14, dans lequel l'alliage de ferrosilicium liquide est fourni directement à partir d'un four de réduction, dans lequel le ferrosilicium est produit tel quel à partir de matières premières selon des procédés classiques.

16. Procédé selon la revendication 14, dans lequel l'alliage de ferrosilicium liquide est fourni par refusion d'une charge d'alliage de ferrosilicium.

17. Procédé selon l'une quelconque des revendications 14 à 16, dans lequel la matière première contenant de l'oxyde de vanadium est une ou plusieurs phases d'oxyde de vanadium choisies parmi l'oxyde de vanadium(II), l'oxyde de vanadium(III), l'oxyde de vanadium(IV), l'oxyde de vanadium(V) et/ou d'autres oxydes non principaux de vanadium et/ou la matière première contenant de l'oxyde de niobium est une ou plusieurs phases d'oxyde de niobium choisies parmi l'oxyde de niobium(II), l'oxyde de niobium(III), l'oxyde de niobium(IV), l'oxyde de niobium(V) et/ou d'autres oxydes non principaux de niobium.

18. Procédé selon la revendication 17, dans lequel la phase d'oxyde de vanadium est l'oxyde de vanadium (V), V₂O₅ et/ou l'oxyde de vanadium(III), V₂O₃ et/ou la phase d'oxyde de niobium est l'oxyde de niobium(V), Nb₂O₅ et/ou l'oxyde de niobium(III), Nb₂O₃.

19. Procédé selon la revendication 17 ou 18, dans lequel la matière première contenant de l'oxyde de vanadium comprend en outre un déchet industriel ou un minerai comprenant du vanadium élémentaire ou de l'oxyde de vanadium, et/ou la matière première contenant de l'oxyde de niobium comprend en outre un déchet industriel ou un minerai comprenant du niobium élémentaire ou de l'oxyde de niobium.

20. Procédé selon l'une quelconque des revendications 14 à 19, comprenant en outre l'ajout d'un composé modificateur de scories à l'alliage de ferrosilicium liquide en une quantité de 0,5 à 30 % en poids, par rapport à la quantité totale d'alliage de ferrosilicium.

21. Procédé selon la revendication 20, dans lequel le composé modificateur de scories est au moins l'un parmi CaO et MgO.

22. Procédé selon l'une quelconque des revendications 14 à 21, dans lequel l'alliage de ferrosilicium liquide de départ a une composition générale :
45 à 90 % en poids de Si ;
jusqu'à 0,5 % en poids de C ;
jusqu'à 2 % en poids d'Al ;
jusqu'à 1,5 % en poids de Ca ;
jusqu'à 0,1 % en poids de Ti ;
jusqu'à 26 % en poids de Mn ;
jusqu'à 26 % en poids de Cr ;
jusqu'à 0,02 % en poids de P ;
jusqu'à 0,005 % en poids de S ;
le reste étant du Fe et des impuretés accidentelles.

23. Procédé selon l'une quelconque des revendications 14 à 22, comprenant en outre l'ajout d'aluminium à la masse fondue de ferrosilicium, avant, simultanément ou après l'ajout de la matière première contenant de l'oxyde de vanadium et/ou de la matière première contenant de l'oxyde de niobium, en une quantité allant jusqu'à 10 % en poids, sur la base de la quantité totale de ferrosilicium et d'oxyde de vanadium et/ou d'oxyde de niobium.

24. Procédé selon l'une quelconque des revendications 14 à 23, comprenant le mélange de l'alliage de ferrosilicium liquide et de la matière première contenant de l'oxyde de vanadium et/ou de la matière première contenant de l'oxyde de niobium, et de tout composé modificateur d'aluminium et/ou de scories ajouté, par agitation mécanique ou agitation gazeuse.

25. Procédé selon l'une quelconque des revendications 14 à 24, dans lequel les scories sont séparées avant ou pendant la coulée de l'alliage liquide FeSi V et/ou Nb.

26. Procédé selon l'une quelconque des revendications 14 à 25, comprenant en outre le broyage et éventuellement le calibrage en fractions granulométriques de l'alliage FeSi V et/ou Nb solidifié ou coulé.

27. Utilisation d'un alliage FeSi V et/ou Nb, selon l'une quelconque des revendications 1 à 13, comme additif dans la fabrication d'aciers contenant du vanadium et/ou du niobium.

28. Utilisation selon la revendication 27, dans laquelle les aciers contenant du vanadium et/ou du niobium sont choisis parmi les aciers pour ressorts, les aciers pour outils, les aciers pour forgeage, les aciers pour rails, les aciers pour barres d'armature, les aciers pour tôles fortes, les aciers automobiles microalliés et les aciers pour avions.
